

May 6, 1930.

W. FONDILLER

1,757,710

ELECTROMAGNETIC CIRCUITS AND APPARATUS

Filed Dec. 17, 1926



Fig. 2



Inventor:  
William Fondiller,  
by E. V. Briggs  
Attorney

## UNITED STATES PATENT OFFICE

WILLIAM FONDILLER, OF YONKERS, NEW YORK, ASSIGNOR TO WESTERN ELECTRIC COMPANY, INCORPORATED, OF NEW YORK, N. Y., A CORPORATION OF NEW YORK

## ELECTROMAGNETIC CIRCUITS AND APPARATUS

Application filed December 17, 1926. Serial No. 155,513.

This invention relates to electromagnetic circuits and apparatus, particularly to their application in signaling systems.

An object of the invention is to secure constancy of operating characteristics in electromagnetic circuits and apparatus employing low field strengths.

A related object of the invention is to reduce distortion due to energy dissipation and intermodulation in signaling systems.

It is well known that when iron and most magnetic compositions of iron are subjected to magnetic fields set up by signaling currents, the permeability and hysteresis losses vary appreciably with changes in the field strength or in the resultant flux density. Such variations in magnetic characteristics produce distortion in the signaling currents, which is variously characterized as modulation, flutter effect, etc., depending upon the conditions under which it is produced.

The present invention relates particularly to magnetic circuits containing cobalt steel alloys which exhibit relative constancy of magnetic characteristics over a range of magnetizing forces including the forces ordinarily employed in signaling. These compositions have heretofore been used extensively for permanent magnets because of their high coercivity at large magnetizing forces, but according to the present invention are used in circuits employing low magnetizing forces, in which region these alloys have been found to exhibit low coercivity with accompanying constant permeability and low hysteresis loss.

The characteristics of substantially constant permeability and low hysteresis loss exhibited by these alloys in the range of magnetizing forces below five gauss render them especially serviceable as the core material for transformers, loading coils, filter inductance coils, sensitive electrical measuring instruments, etc., where uniformity of characteristics over the operating range is demanded.

The advantage of obtaining a constant inductance with resulting low energy dissipation and wave distortion is obvious to those skilled in the art.

The invention will be described in connec-

tion with the accompanying drawing in which:

Fig. 1 is a diagrammatic illustration of a carrier wave telephone system containing magnetic elements in accordance with the invention; and

Fig. 2 is a magnetization curve of a particular cobalt steel alloy which may be employed as the core material in the electromagnetic circuits of Fig. 1.

Fig. 1 shows the west terminal of a carrier wave telephone system connected to the multiplex transmission line ML. The usual east terminal, which is similar to the west terminal, is omitted for the sake of simplifying the showing. A system of this general type is illustrated in Fig. 42 of an article entitled "Carrier current telephony and telegraphy" by Messrs. Colpitts and Blackwell, published in the Transactions of the American Institute of Electrical Engineers, vol. 40, 1921.

The terminal apparatus includes a plurality of transmitting and receiving channels of which the transmitting channel TC and the receiving channel RC are typical. The channel TC includes a modulator M, an oscillator O and a band filter F, and the channel RC includes a demodulator amplifier DA and a band filter F'. These channels are connected to a low frequency telephone line L by means of a special balanced transformer H and balancing network N. The band filters F and F' are of the well known type disclosed in U. S. Patent No. 1,227,113 to G. A. Campbell, issued May 22, 1917, and comprise a plurality of inductance coils and condensers arranged to pass with negligible attenuation waves comprised within predetermined bands of frequencies, and substantially to suppress waves of all other frequencies. The multiplex transmission line ML is loaded at suitable intervals by means of loading coils C, only one of which is shown in the drawing.

Carrier waves are utilized for transmission over the line ML, a separate band of frequencies being allotted to each channel. Voice frequency waves originating in the low frequency line L pass through the balanced transformer H into the modulator M where

55

60

65

70

75

80

85

90

95

100

they are combined with carrier waves from the oscillator O. Of the components of modulation appearing in the output circuit of the modulator, the band filter F may suppress all but one sideband and the carrier, which it passes to the multiplex line ML. In receiving signals, the incoming carrier and sideband waves assigned to the channel RC are selectively passed by the band filter F' and demodulated and amplified in the demodulator-amplifier DA. The voice frequency components of demodulation appearing in the output circuit of the demodulator-amplifier DA are transmitted through balanced transformer coil H to the low frequency line L.

The apparatus which may employ the magnetic cobalt steel alloys as the core material, according to the invention, are the balanced transformer H, the inductance coils 20 of the filters F and F' and the loading coil C. Heretofore, it has been necessary in some cases to construct such apparatus with air cores because of the hysteresis loss and the variations in permeability attendant upon 25 the use of iron and other commonly used magnetic materials. Variations in these magnetic characteristics due to slight change in magnetizing force produce serious distortion in the signaling waves which 30 greatly impairs the transmission efficiency of the system. According to this invention, stability of magnetic characteristics is obtained by employing a hard magnetic steel alloy containing carbon, iron, cobalt and 35 other elements as the core material in the electromagnetic field. Alloys suitable for this purpose have been upon the market under the trade name of KS steel.

The magnetization curve of Fig. 2 illustrates the relation between the magnetizing force H and the induced flux indensity B in c. g. s. units, for an alloy containing 35% cobalt, 7% tungsten, 2% chromium, .7% carbon and the remainder iron. This relation 40 is linear over the range of magnetizing forces from zero to about 5 gauss, the permeability being approximately 10.9, over this range. Tests on another representative sample of this material were confined to the 45 range of magnetizing forces from 0.022 gauss to 0.10 gauss, which includes the range of magnetizing forces ordinarily employed in signaling, this sample having a permeability of about 21 over this range. This 50 latter sample was previously given a supplementary heat treatment which accounts for its higher permeability. The coercivity and hysteresis loss in each case are low. Other suitable cobalt steel alloys are disclosed in 55 U. S. Patents Nos. 1,338,132 and 1,338,133 to K. Honda, issued April 27, 1920. By employing these magnetic materials for the magnetic cores in the magnetic circuits of Fig. 1 the transmission efficiency of the system is greatly improved.

If apparatus containing solid cores of these alloys were used at high frequency, magnetizing forces, relatively large losses due to eddy currents would result. In order to reduce such eddy current losses the core material may be constructed in powder form, employing a suitable insulating material between the particles.

The invention is capable of other modifications and adaptations not specifically described but included within the scope of the appended claims. For example, other steel alloys exhibiting similar properties may be employed in place of cobalt steel, the term "steel" used in the claims referring to an alloy of iron in which carbon is an essential element.

The invention claimed is:

1. The combination with a magnetic material comprising a steel alloy consisting chiefly of iron and cobalt having substantially constant permeability at low magnetizing forces, of a magnetic circuit containing said material, and means for impressing upon said circuit a plurality of small magnetizing force components corresponding respectively to components of a composite signaling wave.

2. The combination with a magnetic material comprising a cobalt steel alloy containing from 5% to 60% cobalt and the balance chiefly iron, having substantially constant permeability at low magnetizing forces, of a magnetic circuit containing said material, and means for impressing upon said circuit a plurality of small magnetizing force components corresponding respectively to components of a composite signaling wave.

3. The combination with a magnetic material comprising a steel alloy consisting chiefly of iron and cobalt having substantially constant permeability over a range of low magnetizing forces, of a magnetic circuit containing said material, and means for impressing upon said circuit a plurality of small magnetizing force components not exceeding the value at which the permeability of the magnetic material begins to vary substantially.

4. A signaling system comprising an inductance the field of which contains a magnetic steel alloy consisting chiefly of iron and cobalt having substantially constant permeability over a range of low magnetizing forces, and a circuit for impressing upon said inductance a plurality of small magnetizing force components comprised within said range.

5. A signaling system comprising a circuit for transmitting waves of different frequencies, and a filter for selectively passing certain of said waves, said filter comprising an inductance the field of which contains a magnetic steel alloy consisting chiefly of iron and cobalt and having substantially constant per-

meability at magnetizing forces of the order impressed upon said circuit.

6. A signaling system comprising a circuit for transmitting waves of different frequencies, and a filter for selectively passing certain of said waves, said filter comprising an inductance the field of which includes a cobalt steel alloy containing from 5% to 60% cobalt and the balance chiefly iron and having substantially constant permeability at magnetizing forces from zero to approximately five gauss.

In witness whereof, I hereunto subscribe my name this 17th day of December, A. D. 1926.

15 WILLIAM FONDILLER.

20

25

30

35

40

45

50

55

60

65